# EUROPEAN PATENT SPECIFICATION

(11) **EP 0 064 167 B1**
(45) Date of publication and mention of the grant of the patent: **21.11.1985**
(21) Application number: 82102964.2
(22) Date of filing: 07.04.1982
(51) Int. Cl.: D01F 6/04

(54) **Process for producing high tenacity, high modulus crystalline thermoplastic article and novel product fibers**
Verfahren zur Herstellung eines thermoplastischen kristallinen Gegenstandes mit hoher Festigkeit und hohem Modulus und Faserprodukte
Procédé pour la fabrication d'un article thermoplastique cristallin ayant une haute ténacité et un module élevé et produits fibreux fabriqués utilisant le procédé

(30) Priority: 30.04.1981 US 259266; 19.03.1982 US 359019; 19.03.1982 US 359020
(43) Date of publication of application: 10.11.1982
(73) Proprietor: ALLIED CORPORATION, Morristown New Jersey 07960 (US)
(72) Inventor: Kavesh, Sheldon, Whippany New Jersey 07981 (US); Prevorsek, Dusan Ciril, Morristown New Jersey 07960 (US)
(74) Representative: Baillie, Iain Cameron

## Description

### Background of the invention

The present invention relates to crystalline thermoplastic articles such as fibers or films having high tenacity, modulus and toughness values and a process for their production which includes a gel intermediate.

The preparation of high strength, high modulus polyethylene fibers by growth from dilute solution has been described by U.S. Patent 4,137,394 to Meihuizen et al. (1979) and U.S. Patent 4,356,138 to Kavesh et al. (1982). Fibers so produced have unacceptably high creep values (over 5% creep after 50 days at 23°C at 10% of breaking load).

GB―A―2,042,414 of Smith and Lemstra describes a process in which a dilute solution of ultrahigh molecular weight polyethylene (UHMWPE) is spun into a quench bath where a gel fiber (still dilute in UHMWPE) is formed. The wet gel (98% solvent in the Examples) was hot-stretched and simultaneously dried of the solvent (see page 1, line 102-page 2, line 1). Decalin is used in the Examples.

The product UHMWPE fiber of GB-A-2,042,414 is described as having, at maximum stretch ratio, a tenacity of 3.02 GPa and a modulus of 90.2 GPa. An article by the named inventors in J. Mat. Sci., vol. 15, pp. 505-514 (1980) describes the same process and essentially the same example (compare Table 1 at page 509 of the article to Table 1 at page 3 of GB-A-2,042,414) and indicates (on page 510 and in Figure 10) that the peak melting temperature (by DSC at 10°C/minute heating rate) reached asymtotically a value of 145.5°C at a draw ratio of 31.7.

The product polypropylene fibers of GB-A-2,042,414 had weight average molecular weights of 1,500,000 and 3,000,000 and tensile strengths of 1.56 GPa and 1 GPa. No moduli or melting temperatures are reported.

In GB-A-2,051,667 the same named inventors describe a process spinning a solution of UHMWPE in a solvent whose boiling point is at least equal to the spinning temperature, but not so high as to render it difficult to evaporate it from the spun filaments (e.g., decalin). Various combinations of evaporation of solvent upon spinning and extraction are contemplated (page 2, lines 66-84) but Examples l―lll compare three spinning procedures: (I) evaporating from 98% solvent to over 90% solvent, (II) evaporating from 98% solvent to 6% solvent by using hot air and (III) evaporating with hot air to 6% solvent followed by extracting with methanol to no solvent. The moduli obtainable (Figure 1) exceeded 80 GPa when the filament entering the drawing step exceeded 90% solvent (open circles), exceeded 70 GPa when the filament entering the drawing step was 6% solvent (closed circles) and remained under 45 GPa when the filament entering the drawing step has been extracted with methanol (see conclusions at page 4, lines 1-7). Similarly, in Figure 3, the substantially dry (6% solvent) filaments could be hot stretched to fibers of lesser modulus than filaments containing over 90% solvent.

Smook et al. in Polymer Bull., vol. 2, pp. 775-83 (1980) describe a process in which UHMWPE is dissolved in a nonvolatile solvent (paraffin oil) and the solution is cooled to room temperature to form a gel. The gel is cut into pieces, fed to an extruder and spun into air to form a porous gel filament. The gel filament is extracted with hexane to remove the paraffin oil, vacuum dried and then stretched to form the desired fiber.

Kalb and Pennings in Polymer, vol. 21, pp. 3―4 (1980) describe a process in which a 5% UHMWPE solution in paraffin oil was spun through a conical die (into air), extracted with hexane, dried under vacuum (to form a porous gel fiber) and drawn in a tube with a temperature gradient of 1-0°C to 148°C. The success of the process is described as being based upon a high microporosity of the fiber to be drawn (0.55 cm³ free volume/cm³ porous fiber or 55% porosity). Maximum properties obtained were 3.0 GPa tensile strength, 106 GPa modulus and 6.4% elongation at break.

Other articles describing similar work of Smith and Lemstra or of Pennings and co-workers include the following.
Kalb & Pennings, Polymer Bull., vol. 1, pp. 871-876 (1979);
Smook & Pennings, J. Pol. Sci., vol. 27, pp. 2209-2228 (1982);
Smith & Lemstra, Makromol. Chem., vol. 180, pp. 2983-2986 (1979);
Smith, Lemstra, Kalb & Pennings, Pol. Bull., vol. 1, pp. 733-736 (1979).

### Brief description of the invention

The present invention includes a continuous process for producing a high strength, high modulus fiber or film which comprises the steps: -
a) forming a solution of a thermoplastic crystalline polymer which is polyethylene of weight average molecular weight at least 500,000 or polypropylene of weight average molecular weight at least 750,000, or which is polyoxymethylene, polybutene-1, poly-(vinylidene fluoride) and/or poly(4-methylpentene-1) having a weight average molecular length between 7x10" and 71 x 104 backbone atoms in a first solvent which is non-volatile at a first temperature, the solution having a first concentration by weight of polymer per unit weight of first solvent;
b) extruding said solution through an aperture, said solution being at a temperature not less than said first temperature upstream of the aperture and being substantially at the first concentration both upstream and downstream of the aperture;
c) cooling the emerging stream adjacent to and downstream of the aperture from the first temperature to a second temperature below the temperature at which a rubbery gel stream is formed, including quenching in a quench bath;
d) extracting the first solvent from the gel stream with a second, volatile solvent;
e) drying the gel fiber or film containing second solvent to form a continuous xerogel fiber or film free of first and second solvent; and
f) stretching at least one of:
   (i) the gel stream containing the first solvent from step c,
   (ii) the gel fiber or film containing the second solvent from step d and,
   (iii) the xerogel fiber or film,

   at a total stretch ratio:
   (i) in the case of polyethylene which is sufficient to achieve a tenacity of at least 20 g/denier (1.7 GPa) and a modulus of at least 600 g/denier (51 GPa),
   (ii) in the case of polypropylene which is sufficient to achieve a tenacity of at least 10 g/denier (0.8 GPa) and a modulus of at least 180 g/denier (14 GPa), and
   (iii) in the case of polyoxymethylene, polybutene-1, poly(vinylidene fluoride) or poly(4-methylpentene-1 ) of at least 10:1.

The present invention also includes a continuous polyethylene fiber of weight average molecular weight at least 500,000 and having a tenacity of at least 20 g/denier (1.7 GPa) and a tensile modulus at least 500 g/denier (43 GPa), characterized by having a creep value no more than 5% (when measured at 10% of breaking load for 50 days at 23°C), a porosity less than 10% and a main melting temperature of at least 147°C (measured by DSC at 10°C/minute heating rate).

The present invention also includes a continuous polypropylene fiber of weight average molecular weight at least 750,000 and having a tenacity of at least 8 g/denier (0.6 GPa), characterized by having a tensile modulus of at least 160 g/denier (13.7 GPa) and a main melting temperature of at least 168°C (measured by DSC at 10°C/minute heating rate).

The present invention also includes a continuous polyolefin gel fiber comprising between 4 and 20 weight % solid polyethylene of weight average molecular weight at least 500,000 or solid polypropylene of weight average molecular weight at least 750,000, and between 80 and 96 weight % of a swelling solvent miscible with high boiling hydrocarbon and having an atmospheric boiling point less than 50°C.

### Brief description of the drawing

Figure 1 is a graphic view of the tenacities of polyethylene fibers prepared accordingly to Examples 3-99 of the present invention versus calculated values therefore as indicated in the Examples. The numbers indicated multiple points.
Figure 2 is a graphic view of the calculated tenacities of polyethylene fibers prepared according to the present invention as a function of polymer concentration and draw ratio at a constant temperature of 140°C.
Figure 3 is a graphic view of the calculated tenacities of polyethylene fibers prepared according to the present invention as a function of draw temperature and draw (or stretch) ratio at a constant polymer concentration of 4%.
Figure 4 is a graphic view of tenacity plotted against tensile modulus for polyethylene fibers prepared in accordance with the present invention.
Figure 5 is a schematic view of a first process embodiment of the present invention.
Figure 6 is a schematic view of the second process embodiment of the present invention.
Figure 7 is a schematic view of a third process embodiment of the present invention.

### Detailed description of the invention

There are many applications which require a load bearing element of high strength, modulus, toughness, dimensional and hydrolytic stability and high resistance to creep under sustained loads.

For example, marine ropes and cables, such as the mooring lines used to secure supertankers to loading stations and the cables used to secure deep sea drilling platforms to underwater anchorage, are presently constructed of materials such as nylon, polyester, aramids and steel which are subject to hydrolytic or corrosive attack by sea water. In consequence such mooring lines and cables are constructed with significant safety factors and are replaced frequently. The greatly increased weight and the need for frequent replacement create substantial operational and economic burdens.

The fibers and films of this invention are of high strength, extraordinarily high modulus and great toughness. They are dimensionally and hydrolytically stable and resistant to creep under sustained loads.

The fibers and films of the invention prepared according to the present process possess these properties in a heretofore unattained combination, and are therefore quite novel and useful materials.

Other applications for the fibers and films of this invention include reinforcements in thermoplastics, thermosetting resins, elastomers and concrete for uses such as pressure vessels, hoses, power transmission belts, sports and automotive equipment, and building construction.

In comparison to the prior art fibers prepared by Smith, Lemstra and Pennings described in DE-A-30 04 699, GB-A-205,1667 and other cited references, the strongest fibers of the present invention are of higher melting point, higher tenacity and much higher modulus. Additionally, they are more uniform, and less porous than the prior art fibers.

In comparison with DE-A-30 04 699 to Smith et. al. the process of the present invention has the advantage of greater controllability and reliability in that the steps of drying and stretching may be separate and each step may be carried out under optimal conditions. To illustrate, Smith & Lemstra in Polymer Bulletin, vol. 1, pp. 733-36 (1979) indicate that drawing temperature, below 143°C, had no effect on the relationships between either tenacity or modulus and stretch ratio. As will be seen, the properties of the fibers of the present invention may be controlled in part by varying stretch temperature with other factors held constant.

In comparison with the procedure described by Smook et. al. in Polymer Bulletin, vol. 2, pp. 775-83 (1980) and in the above Kalb and Pennings articles, the process of the present invention has the advantage that the intermediate gel fibers which are spun are of uniform concentration and this concentration is the same as the polymer solution as prepared. The advantages of this uniformity are illustrated by the fact that the fibers of the present invention may be stretched in a continuous operation to prepare packages of indefinite length. Additionally, the intermediate xerogel fibers of the present invention preferably contain less than 10 volume % porosity compared to 23-65% porosity in the dry gel fibers described by Smook et a/. and Kalb and Pennings.

The crystallizable polymer used in the present invention may be a polyolefin such as polyethylene, polypropylene or poly(methylpentene-1) or may be another polymer such as poly(oxymethylene) or poly(vinylidene fluoride). In the case of polyethylene, suitable polymers have molecular weights (by intrinsic viscosity) in the range of one to ten million. This corresponds to a weight average chain length of 3.6x 10⁴ to 3.6x10⁵ monomer units or 7x 10⁴ to 7.1x10⁵ carbons. Other polyolefins and poly(haloolefins) should have similar backbone carbon chain lengths. For polymers such as poly(oxymethylene) the total chain length should preferably be in the same general range, i.e. 7x10⁴ to 71_{X}10⁴ atoms, with some adjustment possible due to the differences in bond angles between C-C-C and C-0-C.

The weight average molecular weight of polyethylene used is at least 500,000 (6 IV), preferably at least 1,000,000 (10 IV), and more preferably between 2,000,000 (16 IV) and 8,000,000 (42 IV). The weight average molecular weight of polypropylene used is at least 750,000 (5 IV), preferably at least 1,000,000 (6 IV), more preferably at least 1,500,000 (9 IV) and most preferably between 2,000,000 (11 IV) and 8,000,000 (33 IV). The IV numbers represent intrinsic viscosity of the polymer in decalin at 135°C.

The first solvent should be non-volatile under the processing conditions. This is necessary in order to maintain essentially constant the concentration of solvent upstream and through the aperture (die) and to prevent non-uniformity in liquid content of the gel fiber or film containing first solvent. Preferably, the vapor pressure of the first solvent should be no more than 20 kPa (one-fifth of an atmosphere) at 175°C, or at the first temperature. Preferred first solvents for hydrocarbon polymers are aliphatic and aromatic hydrocarbons of the desired non-volatility and solubility for the polymer. The polymer may be present in the first solvent at a first concentration which is selected from a relatively narrow range, e.g. 2 to 15 weight percent, preferably 4 to 10 weight percent and more preferably 5 to 8 weight percent; however, once chosen, the concentration should not vary adjacent the die or otherwise prior to cooling to the second temperature. The concentration should also remain reasonably constant over time (i.e. length of the fiber or film).

The first temperature is chosen to achieve complete dissolution of the polymer in the first solvent. The first temperature is the minimum temperature at any point between where the solution is formed and the die face, and must be greater than the gelation temperature for the polymer in the solvent at the first concentration. For polyethylene in paraffin oil at 5-15% concentration, the gelation temperature is approximaely 100-130°C; therefore, a preferred first temperature can be between 180°C and 250°C, more preferably 200-240. While temperatures may vary above the first temperature at various points upstream of the die face, excessive temperatures causitive of polymer degradation should be avoided. To assure complete solubility, a first temperature is chosen whereat the solubility of the polymer exceeds the first concentration, and is typically at least 100% greater. The second temperature is chosen whereas the solubility of the polymer is much less than the first concentration. Preferably, the solubility of the polymer in the first solvent at the second temperature is no more than 1 % of the first concentration. Cooling of the extruded polymer solution stream from the first temperature to the second temperature should be accomplished at a rate sufficiently rapid to form a gel fiber which is of substantially the same polymer concentration as existed in the polymer solution. Preferably the rate at which the extruded polymer solution stream is cooled from the first temperature to the second temperature should be at least 50°C per minute.

Some stretching during cooling to the second temperature is not excluded from the present invention, but the total stretching during this stage should not normally exceed 2:1, and preferably no more than 1.5:1. As a result of those factors the gel fiber formed upon cooling to the second temperature consists of a continuous polymeric network highly swollen with solvent. The gel usually has regions of high and low polymer density on a microscopic level but is generally free of large (greater than 500 nm) regions void of solid polymer.

If an aperture of circular cross section (or other cross section without a major axis in the plane perpendicular to the flow direction more than 8 times the smallest axis in the same plane, such as oval, Y-or X-shaped aperture) is used, then both gels will be gel fibers, the xerogel will be an xerogel fiber and the final product will be a fiber. The diameter of the aperture is not critical, with representative apertures being between 0.25 mm and 5 mm in diameter (or other major axis). The length of the aperture in the flow direction should normally be at least 10 times the diameter of the aperture (or other similar major axis), preferably at least 15 times and more preferably at least 20 times the diameter (or other similar major axis).

If an aperture of rectangular cross section is used, then both gels will be gel films, the xerogel will be a xerogel film and the final product will be a film. The width and height of the aperture are not critical, with representative apertures being between 2.5 mm and 2 m in width (corresponding to film width), between 0.25 mm and 5 mm in height (corresponding to film thickness). The depth of the aperture (in the flow direction) should normally be at least 10 times the height of the aperture, preferably at least 15 times the height and more preferably at least 20 times the height.

The extraction with second solvent is conducted in a manner that replaces the first solvent in the gel with second solvent without significant changes in gel structure. Some swelling or shrinkage of the gel may occur, but preferably no substantial dissolution, coagulation or precipitation of the polymer occurs.

When the first solvent is a hydrocarbon, suitable second solvents include hydrocarbons, chlorinated hydrocarbons, chlorofluorinated hydrocarbons and others, such as pentane, hexane, heptane, toluene, methylene chloride, carbon tetrachloride, trichlorotrifluoroethane (TCTFE), diethyl ether and dioxane.

The most preferred second solvents are methylene chloride (B.P. 39.8°C) and TCFE (B.P. 47.5°C). Preferred second solvents are the non-flammable volatile solvents having an atmospheric boiling point below 80°C, more preferably below 70°C and most preferably below 50°C. Conditions of extraction should remove the first solvent to less than 1% of the total solvent in the gel.

A preferred combination of conditions is a first temperature between 150°C and 250°C, a second temperature between -40°C and 40°C and a cooling rate between the first temperature and the second temperature of at least 50°C/minute. It is preferred that the first solvent be a hydrocarbon, when the polymer is a polyolefin such as ultrahigh molecular weight polyethylene. The first solvent should be substantially non-volatile, one measure of which is that its vapor pressure at the first temperature should be less than one-fifth atmosphere (20 kPa), and more preferably less than 2 kPa.

In choosing the first and second solvents, the primary desired difference relates to volatility as discussed above. It is also preferred that the polymers be less soluble in the second solvent at 40°C than in the first solvent at 150°C.

Once the gel containing second solvent is formed, it is then dried under conditions where the second solvent is removed leaving the solid network of polymer substantially intact. By analogy to silica gels, the resultant material is called herein a "xerogel" meaning a solid matrix corresponding to the solid matrix of a wet gel, with the liquid replaced by gas (e.g. by an inert gas such as nitrogen or by air). The term "xerogel" is not intended to delineate any particular type of surface area, porosity or pore size.

A comparison of the xerogels of the present invention with corresponding dried gel fibers prepared according to prior art indicates the following major differences in structure: The dried xerogel fibers of the present invention preferably contain less than ten volume percent pores compared to approximately 55 volume percent pores in the Kalb and Pennings dried gel fibers and approximately 23-65 volume percent pores in the Smook et a/. dried gel fibers. The dried xerogel fibers of the present invention show a surface area (by the B.E.T. technique) of less than 1 m²/g as compared to 28.8 m²/g in a fiber prepared by the prior art method (see Comparative Example 1 and Example 2, below).

The xerogel fibers of the present invention are also novel compared to dry, unstretched fibers of GB-A-2,051,667 and DE-A-3004699 and related articles by Smith and Lemstra. This difference is evidenced by the deleterious effect of stretching below 75°C or above 135°C upon the Smith and Lemstra unstretched fibers. In comparison, stretching of the present xerogel fibers at room temperature and above 135°C has beneficial rather than deleterious effects (see, for example, Examples 540-542, below). While the physical nature of these differences are not clear because of lack of information about Smith and Lemstra's unstretched fibers, it appears that one or more of the following characteristics of the present xerogel fibers must be lacking in Smith and Lemstra's unstretched fibers: (1) a crystalline orientation function less than 0.2, and preferably less than 0.1 as measured by wide angle X-ray diffraction; (2) microporosity less than 10% and preferably less than 3%; (3) a crystallinity index as measured by wide angle X-ray diffraction (see P. H. Hermans and A. Weidinger, Macromol. Chem. vol. 44, p. 24 (1961)) less than 80% and preferably less than 75%; (4) no detectable fraction of the triclinic crystalline form and (5) a fractional variation of the spherulite size across a diameter of the fiber less than 0.25.

Stretching may be performed upon the gel fiber after cooling to the second temperature or during or after extraction. Alternatively, stretching of the xerogel fiber may be conducted, or a combination of gel stretch and xerogel stretch may be performed. The stretching may be conducted in a single stage or it may be conducted in two or more stages. The first stage stretching may be conducted at room temperatures or at an elevated temperature. Preferably the stretching is conducted in two or more stages with the last of the stages performed at a temperature between 120°C and 160°C. Most preferably the stretching is conducted in at least two stages with the last of the stages performed at a temperature between 135°C and 150°C. The Examples, and especially Examples 3-99 and 111-486, illustrate how the stretch ratios can be related to obtaining particular fiber properties.

The product polyethylene fibers produced by the present process represent novel articles in that they include fibers with a unique combination of properties: a modulus at least 500 g/denier (preferably at least 1000 g/denier, more preferably at least 1600 g/denier and most preferably at least 2000 g/denier), a tenacity at least 20 g/denier (preferably at least 30 g/denier and more preferably at least 40 g/denier), a main melting temperature of at least 147°C (preferably at least 149°C), measured at 10°C/minute heating rate by differential scanning calorimetry, a porosity of no more than 10% (preferably no more than 6%) and a creep value no more than 5% (preferably no more than 3%) when measured a 10% of breaking load for 50 days at 23°C. Preferably the fiber has an elongation to break at most 7%. In addition, the fibers have high toughness and uniformity. Furthermore, as indicated in Examples 3-99 and 111-489 below, trade-offs between various properties can be made in a controlled fashion with the present process.

The novel polypropylene fibers of the present invention also include a unique combination of properties, previously unachieved for polypropylene fibers: a tenacity of at least 8 g/denier (preferably at least 11 g/denier and more preferably at least 13 g/denier), a tensile modulus at least 160 g/denier (preferably at least 200 g/denier), a main melting temperature at least 168°C (preferably at least 170°C) measured at 10°C/minute heating rate by differential scanning calorimetry and a porosity less than 10% (preferably no more than 5%). Preferably, the polypropylene fibers also have an elongation to break less than 20%.

Additionally a novel class of fibers of the invention are polypropylene fibers possessing a modulus of at least 200 g/denier, preferably at least 220 g/denier.

The gel fibers containing first solvent, gel fibers containing second solvent and xerogel fibers of the present invention also represent novel articles of manufacture, distinguished from somewhat similar products described by Smook et al. and by Kalb and Pennings in having volume porosities of 10% or less compared to values of 23%-65% in the references.

In particular the second gel fibers differ from the comparable prior art materials in having a solvent with an atmospheric boiling point less than 50°C. As indicated by Examples 100-108, below, the uniformity and cylindrical shape of the xerogel fibers improved progressively as the boiling point of the second solvent declined. As also indicated in Examples 100-108 (see Table III), substantially higher tenacity fibers were produced under equivalent drying and stretching conditions by using trichlorotrifluoroethane (boiling point 47.5°C) as the second solvent compared to fibers produced by using hexane (boiling point 68.7°C) as second solvent. The improvement in final fiber is then directly attributable to changes in the second solvent in the second gel fiber. Preferred such second solvents are halogenated hydrocarbons of the proper boiling point such as methylene chloride (dichloromethane) and trichlorotrifluoroethane, with the latter being most preferred.

### Description of the preferred embodiment

Figure 5 illustrates in schematic form a first embodiment of the present invention, wherein the stretching step F is conducted in two stages on the xerogel fiber subsequent to drying step E. In Figure 5, a first mixing vessel 10 is shown, which is fed with an ultra high molecular weight polymer 11 such as polyethylene of weight average molecular weight at least 500,000 and preferably at least 1,000,000, and to which is also fed a first, relatively non-volatile solvent 12 such as paraffin oil. First mixing vessel 10 is equipped with an agitator 13. The residence time of polymer and first solvent in first mixing vessel 10 is sufficient to form a slurry containing some dissolved polymer and some relatively finely divided polymer particles, which slurry is removed in line 14 to an intensive mixing vessel 15. Intensive mixing vessel 15 is equipped with helical agitator blades 16. The residence time and agitator speed in intensive mixing vessel 15 is sufficient to convert the slurry into a solution. It will be appreciated that the temperature in intensive mixing vessel 15, either because of external heating, heating of the slurry 14, heat generated by the intensive mixing, or a combination of the above is sufficiently high (e.g. 200°C) to permit the polymer to be completely dissolved in the solvent at the desired concentration (generally between 6 and 10 percent polymer, by weight of solution). From the intensive mixing vessel 15, the solution is fed to an extrusion device 18, containing a barrel 19 within which is a screw 20 operated by motor 22 to deliver polymer solution at reasonably high pressure to a gear pump and housing 23 at a controlled flow rate. A motor 24 is provided to drive gear pump 23 and extrude the polymer solution, still hot, through a spinnerette 25 comprising a plurality of apertures, which may be circular, X-shaped, or, oval-shaped, or in any of a variety of shapes having a relatively small major axis in the plane of the spinnerette when it is desired to form fibers, and having a rectangular or other shape with an extended major axis in the plane of the spinnerette when it is desired to form films. The temperature of the solution in the mixing vessel 15, in the extrusion device 18 and at the spinnerette 25 should all equal or exceed a first temperature (e.g. 200°C) chosen to exceed the gellation temperature (approximately 100-130°C for polyethylene in paraffin oil). The temperature may vary (e.g. 220°C, 210°C and 200°C) or may be constant (e.g. 220°C) from the mixing vessel 15 to extrusion device 18 to the spinnerette 25. At all points, however, the concentration of polymer in the solution should be substantially the same. The number of apertures, and thus the number of fibers formed, is not critical, with convenient numbers of apertures being 16, 120, or 240.

From the spinnerette 25, the polymer solution stream passes through an air gap 27, optionally enclosed and filled with an inert gas such as nitrogen, and optionally provided with a flow of gas to facilitate cooling. A plurality of gel fibers 28 containing first solvent pass through the air gap 27 and into a quench bath 30, so as to cool the fibers, both in the air gap 27 and in the quench bath 30, to a second temperature at which the solubility of the polymer in the first solvent is relatively low, such that most of the polymer precipitates as a gel material. While some stretching in the air gap 27 is permissible, it is preferably less than 2:1, and is more preferably much lower.

It is preferred that the quench liquid in quench bath 30 be water. While the second solvent may be used as the quench fluid (and quench bath 30 may even be integral with solvent extraction device 37 described below), it has been found in limited testing that such a modification impairs fiber properties.

Rollers 31 and 32 in the quench bath 30 operate to feed the gel fiber through the quench bath, and preferably operate with little or no stretch. In the event that some stretching does occur across rollers 31 and 32, some first solvent exudes out of the fibers and can be collected as a top layer in quench bath 30.

From the quench bath 30, the cool first gel fibers 33 pass to a solvent extraction device 37 where a second solvent, being of relatively low boiling such as trichlorotrifluoroethane, is fed in through line 38. The solvent outflow in line 40 contains second solvent and essentially all of the first solvent brought in with the cool gel fibers 33, either dissolved or dispersed in the second solvent. Thus the second gel fibers 41 conducted out of the solvent extraction device 37 contain substantially only second solvent, and relatively little first solvent. The second gel fibers 41 may have shrunken somewhat compared to the first gel fibers 33, but otherwise contain substantially the same polymer morphology.

In a drying device 45, the second solvent is evaporated from the second gel fibers 41 forming essentially unstretched xerogel fibers 47 which are taken up on spool 52.

From spool 52, or from a plurality of such spools if it is desired to operate the stretching line at a slower feed rate than the take up of spool 52 permits, the fibers are fed over driven feed roll 54 and idler roll 55 into a first heated tube 56, which may be rectangular, cylindrical or other convenient shape. Sufficient heat is applied to the tube 56 to cause the internal temperature to be between 120 and 140°C. The fibers are stretched at a relatively high draw ratio (e.g. 10:1) so as to form partially stretched fibers 58 taken up by driven roll 61 and idler roll 62. From rolls 61 and 62, the fibers are taken through a second heated tube 63, heated so as to be at somewhat higher temperature, e.g. 130-160°C and are then taken up by driven take-up roll 65 and idler roll 66, operating at a speed sufficient to impart a stretch ratio in heated tube 63 as desired, e.g. 2.5: 1. The twice stretched fibers 68 produced in this first embodiment are taken up on take-up spool 72.

With reference to the six process steps of the present invention, it can be seen that the solution forming step A is conducted in mixers 13 and 15. The extruding step B is conducted with device 18 and 23, and especially through spinnerette 25. The cooling step C is conducted in airgap 27 and quench bath 30. Extraction step D is conducted in solvent extraction device 37. The drying step E is conducted in drying device 45. The stretching step F is conducted in elements 52-72, and especially in heated tubes 56 and 63. It will be appreciated, however, that various other parts of the system may also perform some stretching, even at temperatures substantially below those of heated tubes 56 and 63. Thus, for example, some stretching (e.g. 2:1) may occur within quench bath 30, within solvent extraction device 37, within drying device 45 or between solvent extraction device 37 and drying device 45.

A second embodiment of the present invention is illustrated in schematic form by Figure 6. The solution forming and extruding steps A and B of the second embodiment are substantially the same as those in the first embodiment illustrated in Figure 5. Thus, polymer and first solvent are mixed in first mixing vessel 10 and conducted as a slurry in line 14 to intensive mixing device 15 operative to form a hot solution of polymer in first solvent. Extrusion device 18 impells the solution under pressure through the gear pump and housing 23 and then through a plurality of apertures in spinnerette 27. The hot stream 28 pass through air gap 27 and quench bath 30 so as to form cool first gel fibers 33.

The cool first gel fibers 33 are conducted over driven roll 54 and idler roll 55 through a heated tube 57 which, in general, is longer than the first heated tube 56 illustrated in Figure 5. The length of heated tube 57 compensates, in general, for the higher velocity of fibers 33 in the second embodiment of Figure 6 compared to the velocity of xerogel fibers (47) between take-up spool 52 and heated tube 56 in the first embodiment of Figure 5. The fibers 33 are drawn through heated tube 57 by driven take-up roll 59 and idler roll 60, so as to cause a relatively high stretch ratio (e.g. 10:1). The once-stretched first gel fibers 35 are conducted into extraction device 37.

In the extraction device 37, the first solvent is extracted out of the gel fibers by second solvent and the gel fibers 42 containing second solvent are conducted to a drying device 45. There the second solvent is evaporated from the gel fibers; and xerogel fibers 48, being once-stretched, are taken up on spool 52.

Fibers on spool 52 are then taken up by driven feed roll 61 and idler 62 and passed through a heated tube 63, operating at the relatively high temperature of between 130 and 160°C. The fibers are taken up by driven take up roll 65 and idler roll 66 operating at a speed sufficient to impart a stretch in heated tube 63 as desired, e.g. 2.5:1. The twice-stretched fibers 69 produced in the second embodiment are then taken up on spool 72.

It will be appreciated that, by comparing the embodiment of Figure 6 with the embodiment of Figure 5, the stretching step F has been divided into two parts, with the first part conducted in heated tube 57 performed on the first gel fibers 33 prior to extraction (D) and drying (E), and the second part conducted in heated tube 63, being conducted on xerogel fibers 48 subsequent to drying (E).

The third embodiment of the present invention is illustrated in Figure 7, with the solution forming step A, extrusion step B, and cooling step C being substantially identical to the first embodiment of Figure 5 and the second embodiment of Figure 6. Thus, polymer and first solvent are mixed in first mixing vessel 10 and conducted as a slurry in line 14 to intensive mixing device 15 operative to form a hot solution of polymer in first solvent. Extrusion device 18 impells the solution under pressure through the gear pump and housing 23 and then through a plurality of apertures in spinnerette 27. The hot streams 28 pass through air gap 27 and quench bath 30 so as to form cool first gel fibers 33.

The cool first gel fibers 33 are conducted over driven roll 54 and idler roll 55 through a heated tube 57 which, in general, is longer than the first heated tube 56 illustrated in Figure 5. The length of heated tube 57 compensates, in general, for the higher velocity of fibers 33 in the third embodiment of Figure 7 compared to the velocity of xerogel fibers 47 between takeup spool 52 and heated tube 56 in the first embodiment of Figure 5. The first gel fibers 33 are now taken up by driven roll 61 and idler roll 62, operative to cause the stretch ratio in heated tube 57 to be as desired, e.g. 10:1.

From rolls 61 and 62, the once-drawn first gel fibers 35 are conducted into modified heated tube 64 and drawn by driven take up roll 65 and idler roll 66. Driven roll 65 is operated sufficiently fast to draw the fibers in heated tube 64 at the desired stretch ratio, e.g. 2.5:1. Because of the relatively high line speed in heated tube 64, required generally to match the speed of once-drawn gel fibers 35 coming off of rolls 61 and 62, heated tube 64 in the third embodiment of Figure 7 will, in general, be longer than heated tube 63 in either the second embodiment of Figure 6 or the first embodiment of Figure 5. While first solvent may exude from the fiber during stretching in heated tubes 57 and 64 (and be collected at the exit of each tube), the first solvent is sufficiently non-volatile so as not to evaporate to an appreciable extent in either of these heated tubes.

The twice-stretched first gel fibers 36 are then conducted through solvent extraction device 37, where the second, volatile solvent extracts the first solvent out of the fibers. The second gel fibers, containing substantially only second solvent, are then dried in drying device 45, and the twice-stretched fibers 70 are then taken up on spool 72.

It will be appreciated that, by comparing the third embodiment of Figure 7 to the first two embodiments of Figures 5 and 6, the stretching step (F) is performed in the third embodiment in two stages, both subsequent to cooling step C and prior to solvent extracting step D.

The process of the invention will be further illustrated by the examples below. The first example illustrates the prior art techniques of Smook et. al. and the Kalb and Pennings articles.

### Comparative Example 1

A glass vessel equipped with a PTFE paddle stirrer was charged with 5.0 wt% linear polyethylene (sold as Hercules UHMW 1900, having 24 IV and approximately 4x 10⁶ M.W.), 94.5 wt% paraffin oil (J. T. Baker, 345-355 Saybolt viscosity) and 0.5 wt% antioxidant (sold under the trademark lonol).

The vessel was sealed under nitrogen pressure and heated with stirring to 150°C. The vessel and its contents were maintained under slow agitation for 48 hours. At the end of this period the solution was cooled to room temperature. The cooled solution separated into two phases-A "mushy" liquid phase consisting of 0.43 wt% polyethylene and a rubbery gel phase consisting of 8.7 wt% polyethylene. The gel phase was collected, cut into pieces and fed into a 2.5 cm (one inch) Sterling extruder equipped with a 21/1 UD polyethylene-type screw. The extruder was operated at 10 RPM, 170°C and was equipped with a conical single hole spinning die of 1 cm inlet diameter, 1 mm exit diameter and 6 cm length.

The deformation and compression of the gel by the extruder screw caused exudation of paraffin oil from the gel. This liquid backed up in the extruder barrel and was mostly discharged from the hopper end of the extruder. At the exit end of the extruder a gel fiber of approximately 0.7 mm diameter was collected at the rate of 1.6 m/min. The gel fiber consisted of 24-38 wt% polyethylene. The solids content of the gel fiber varied substantially with time.

The paraffin oil was extracted from the extruded gel fiber using hexane and the fiber was dried under vacuum at 50°C. The dried gel fiber had a density of 0.326 g/cm^{3.} Therefore, based on a density of 0.960 for the polyethylene constituent, the gel fiber consisted of 73.2 volume percent voids. Measurement of pore volume using a mercury porosimeter showed a pore volume of 2.58 cm³/g. A B.E.T. measurement of surface area gave a value of 28.8 m²/g.

The dried fiber was stretched in a nitrogen atmosphere within a hot tube of 1.5 meters length. Fiber feed speed was 2 cm/min. Tube temperature was 100°C at the inlet increasing to 150°C at the outlet.

It was found that, because of filament non-uniformity, stretch ratios exceeding 30/1 were not sustainable for periods exceeding 20 minutes without filament breakage.

The properties of the fiber prepared at 30/1 stretch ratio were as follows:
denier-99
tenacity-23 g/d
modulus-980 g/d
elongation at break-3%
work-to-break―6570 in Ihε lin³ (45 M.l/m³),

The following example is illustrative of the present invention:

### Example 2

An oil jacketed double helical (Helicone@) mixer constructed by Atlantic Research Corporation was charged with 5.0 wt% linear polyethylene (Hercules UHMW 1900 having 17 IV and approximately 2.5x 10⁶ M.W.) and 94.5 wt% paraffin oil (J. T. Baker, 345-355 Saybolt viscosity). The charge was heated with agitation at 20 rpm to 200°C under nitrogen pressure over a period of two hours. After reaching 200°C, agitation was maintained for an additional two hours.

The bottom discharge opening of the Helicone mixer was fitted with a single hole capillary spinning die of 2 mm diameter and 9.5 mm length. The temperature of the spinning die was maintained at 200°C.

Nitrogen pressure applied to the mixer and rotation of the blades of the mixer were used to extrude the charge through the spinning die. The extruded uniform solution filament was quenched to a gel state by passage through water bath located at a distance of 33 cm (13 inches) below the spinning die. The gel filament was wound up continuously on a 15.2 cm (6 inch) diameter bobbin at the rate of 4.5 meters/min.

The bobbins of gel fiber were immersed in trichlorotrifluoroethane (fluorocarbon 113 or "TCTFE") to exchange this solvent for paraffin oil as the liquid constituent of the gel. The gel fiber was unwound from a bobbin, and the fluorocarbon solvent evaporated at 22―50°C.

The dried fiber was of 970±100 denier. The density of the fiber was determined to be 950 kg/m³ by the density gradient method. Therefore, based on a density of 960 kg/m³ for the polyethylene constituent, the dried fiber contained one volume percent voids. A B.E.T. measurement of the surface area gave a value less than 1 m²/g.

The dried gel fiber was fed at 2 cm/min into a hot tube blanketed with nitrogen and maintained at 100°C at its inlet and 140°C at its outlet. The fiber was stretched continuously 45/1 within the hot tube for a period of three hours without experiencing fiber breakage. The properties of the stretched fiber were:
denier-22.5
tenacity-37.6 g/d
modulus-1460 g/d
elongation-4.1 %
work-to-break-12,900 in-lbs/in (89 MJ/m³).

### Examples 3-99

A series of fiber samples was prepared following the procedures described in Example 2, but with variations introduced in the following material and process parameters:
a. polyethylene IV (molecular weight)
b. polymer gel concentration
c. stretch temperature
d. fiber denier
e. stretch ratio.

The results of these experiments upon the final fiber properties obtained are presented in Table I. The Polymer intrinsic viscosity values were 24 in Examples 3-49 and 17 in Examples 50-99. The gel concentration was 2% in Examples 26―41, 4% in Examples 3-17, 5% in Examples 42-99 and 6% in Examples 18-25.

In order to determine the relationships of the fiber properties to the process and material parameters, the data of Table I were subjected to statistical analysis by multiple linear regression. The regression equation obtained for fiber tenacity was as follows:
Tenacity, g/d=-₈.₄7+2.00 ^{*} SR+0.491 ^{*} IV+0.0605 ^{*} C ^{*} SR 0.00623 ^{*}T^{*}SR- 0.0156^{*}IV^{*}SR -0.00919 ^{*} SR ^{*} SR where
SR is stretch ratio
IV is polymer intrinsic viscosity in decalin at 135°C, dl/g
C is polymer concentration in the gel, wt%
T is stretch temp. °C.

The statistics of the regression were:
F ratio (6,95)=1₁₈
significance level=₉₉.₉+%
standard error of estimate=3.0 g/d.

A comparison between the observed tenacities and tenacities calculated from the regression equation is shown in Figure 1.

Figures 2 and 3 present response surface contours for tenacity calculated from the regression equation on two important planes.

In the experiments of Examples 3-99, a correlation of modulus with spinning parameters was generally parallel to that of tenacity. A plot of fiber modulus versus tenacity is shown in Figure 4.

It will be seen from the data, the regression equations and the plots of the calculated and observed results that the method of the invention enables substantial control to obtain desired fiber properties and that greater controllability and flexibility is obtained than by prior art methods.

Further, it should be noted that many of the fibers of these examples showed higher tenacities and/or modulus values than had been obtained by prior art methods. In the prior art methods of DE-A-30 04 699 and GB-A-2051667, all fibers prepared had tenacities less than 3.0 GPa (35 g/d) and moduli less than 100 GPa (1181 g/d). In the present instance, fiber examples Nos. 21, 67, 70, 73, 82, 84 and 88 exceeded both of these levels and other fiber examples surpassed on one or the other property.

In the prior art publications of Pennings and coworkers, all fibers (prepared discontinuously) had moduli less than 121 GPa (1372 g/d). In the present instance continuous fiber examples No. 70, 71, 73, 82, 83, 84, 88 and 99 surpassed this level.

The fiber of example 71 was further tested for resistance to creep at 23°C under a sustained load of 10% of the breaking load. Creep is defined as follows: where
B(s) is the length of the test section immediately after application of load
A(s,t) is the length of the test section at time t after application of load, s
A and B are both functions of the loads, while A is also a function of time t.

For comparison, a commercial nylon tire cord (6 denier, 9.6 g/d tenacity) and a polyethylene fiber prepared in accordance with EP-A-56875 by surface growth and subsequent hot stretching (10 denier, 41.5 g/d tenacity) were similarly tested for creep.

The results of these tests are presented in Table II.

It will be seen that the fiber of Example 71 showed 1.4% creep in 50 days at 23°C under the sustained load equal to 10% of the breaking load. By way of comparison, both the commercial nylon 6 tire cord and the surface grown polyethylene fiber showed 5% creep under similar test conditions.

The melting temperatures and the porosities of the fibers of Examples 64, 70 and 71 were determined. Melting temperatures were measured using a DuPont 990 differential scanning calorimeter. Samples were heated in an argon atmosphere at the rate of 10°C/min. Additionally, the melting temperature was determined for the starting polyethylene powder from which the fibers of Examples 64, 70 and 71 were prepared.

Porosities of the fibers were determined by measurements of their densities using the density gradient technique and comparison with the density of a compression molded plaque prepared from the same initial polyethylene powder. (The density of the compression molded plaque was 960 kg/m³).

Porosity was calculated as follows: Results were as follows:

The particular level and combination of properties exhibited by the fiber of Examples 64, 70 and 71, i.e., tenacity at least 30 g/d, modulus in excess of 1000 g/d (86 GPa) and creep (at 23°C and 10% of breaking load) less than 3% in 50 days, main melting temperature of at least 147°C (by DSC at 10°C/min. heating rate) and porosity less than 10% appears not to have been attained heretofore.

The following Examples illustrate the effect of the second solvent upon fiber properties.

### Examples 100-108

Fiber samples were prepared as described in Example 2, but with the following variations. The bottom discharge opening of the Helicone mixer was adapted to feed the polymer solution first to a gear pump and thence to a single hole conical spinning die. The cross-section of the spinning die tapered uniformly at a 7.5° angle from an entrance diameter of 10 mm to an exit diameter of 1 mm. The gear pump speed was set to deliver 5.84 cm'/min. of polymer solution to the die. The extruded solution filament was quenched to a gel state by passage through a water bath located at a distance of 20 cm below the spinning die. The gel filament was wound up continuously on bobbins at the rate of 7.3 meters/min.

The bobbins of gel fiber were immersed in several different solvents at room temperature to exchange with the paraffin oil as the liquid constituent of the gel. The solvents and their boiling points were:

The solvent exchanged gel fibers were air dried at room temperature. Drying of the gel fibers was accompanied in each case by substantial shrinkage of transverse dimensions. Surprisingly, it was observed that the shape and surface texture of the xerogel fibers departed progressively from a smooth cylindrical form in approximate proportion to the boiling point of the second solvent. Thus, the fiber from which diethyl ether had been dried was substantially cylindrical whereas the fiber from which toluene had been dried was "C" shaped in cross-section.

The xerogel fibers prepared using TCTFE and n-hexane as second solvents were further compared by stretching each at 130°C, incrementally increasing stretch ratio until fiber breakage occurred. The tensile properties of the resulting fibers were determined as shown in Table III.

It will be seen that the xerogel fiber prepared using TCTFE as the second solvent could be stretched continuously to a stretch ratio of 49/1, whereas the xerogel fiber prepared using n-hexane could be stretched continuously only to a stretch ratio of 33/1. At maximum stretch ratio, the stretched fiber prepared using TCTFE second solvent was of 39.8 g/d tenacity and of 1580 g/d modulus. This compares to 32.0 g/d tenacity and 1140 g/d modulus obtained using n-hexane as the second solvent.

### Example 110

Following the procedures of Examples 3-99, an 8 wt% solution of isotactic polypropylene of 12.8 intrinsic viscosity (in decalin at 135°C), approximately 2.1 x 10⁶ M.W. was prepared in paraffin oil at 200°C. A gel fiber was spun at 6.1 meters/min. The paraffin oil was solvent exchanged with TCTFE and the gel fiber dried at room temperature. The dried fiber was stretched 25/1 at a feed roll speed of 2 cm/min. Stretching was conducted in a continuous manner for one hour at 160°C.

Fiber properties were as follows:
denier-105
tenacity-9.6 g/d
modulus-164 g/d
elongation-11.5%
work-to-break-9280 in Ibs./in³ (64 MJ/m³).

### Examples 111-486

A series of xerogel fiber samples was prepared as in Example 2 but using a gear pump to control melt flow rate. Variations were introduced in the following material and process parameters:
a. polyethylene IV (molecular weight)
b. polymer gel concentration
c. die exit diameter
d. die included angle (conical orifice)
e. spinning temperature
f. melt flow rate
g. distance to quench
h. gel fiber take-up velocity
i. xerogel fiber denier.

Each of the xerogel fiber samples prepared was stretched in a hot tube of 1.5 meter length blanketed with nitrogen and maintained at 100°C at the fiber inlet and 140°C at the fiber outlet. Fiber feed speed into the hot tube was 4 cm/min. (Under these conditions the actual fiber temperature was within 1°C of the tube temperature at distances beyond 15 cm from the inlet). Each sample was stretched continuously at a series of increasing stretch ratios. The independent variables for these experiments are summarized below:

### Polymer intrinsic viscosity (dUg)

11.5 - Examples 172-189, 237-241, 251-300, 339-371
15.5 - Examples 111-126, 138―140, 167-171, 204―236, 242―243, 372―449, 457―459
17.7 - Examples 127-137, 141-166, 190-203, 244-250, 301-338
20.9 - Examples 450-456, 467-486

### . Gel concentration

5% - Examples 127-137, 141-149, 167-171, 190―203, 244―260, 274―276, 291―306, 339―371
6% - Examples 111-126, 138―140, 204-236, 242-243, 372-418, 431-486
7% - Examples 150-166, 172-189, 237-241, 261-273, 277-290, 307-338

### Die angle (degrees)

0° - Examples 127-137, 141-149, 261-281, 307-316, 339-365, 419-430
7.5° - Examples 111-126, 138-140, 167―171, 204―243, 251―260, 301―306, 317―338, 372―418, 431-486
15° - Examples 150-166, 172-203, 244-250, 282-300, 366-371

### Spinning temperature

180°C - Examples 172-203, 237-241, 301-322, 339-371
200°C - Examples 111-126, 138-140, 167-171, 204-236, 242-243, 372-486
220°C - Examples 127-137, 141-166, 244-300, 232-338

### Solution flow rate (cm³/min)

2.92±0.02 - Examples 116-122, 135-145, 150-152, 162-166, 172-173, 196-201, 214-222, 237, 240, 242-245, 251-255, 260-265, 277-284, 288-293, 301, 304-306, 310-312, 318―320, 347―360, 368―370, 372, 395―397, 401―407, 412―414, 419―424, 450―459, 467-481
4.37±0.02 - Examples 204-208, 230-236, 377-379, 408―411
5.85±0.05 - Examples 111-115, 123-134, 146-149, 153-161, 167-171, 180-195, 202-203, 209―213, 223―229, 238―239, 241, 256―259, 266―276, 285―287, 294―300, 302―303, 307―309, 315―317, 321―326, 335―338, 361―367, 371, 373―376, 392―394, 398―400, 415―418, 431-433, 482-486
6.07 - Examples 339-346
8.76 - Examples 380-391
8.88 - Examples 246-250
11.71±0.03― Examples 434-437, 445-449
17.29 - Examples 438-440

Under all of the varied conditions, the take-up velocity varied from 90-1621 cm/min, the xerogel fiber denier from 98-1613, the stretch ratio from 5-174, the tenacity from 9―45 g/denier, the tensile modulus from 218-1700 g/denier and the elongation from 2.5-29.4%.

The results of each Example producing a fiber of at least 30 g/denier (2.5 GPa) tenacity or at least 1000 g/denier (86 GPa) modulus are displayed in Table IV. The tenacity and modulus values are expressed in g/den, which can be converted to GPa by multiplying by 0.086 (GPa)/(g/den).

In order to determine the relationships of the fiber properties to the process and material parameters, all of the data from Example 111-486, including those Examples listed in Table IV, were subjected to statistical analysis by multiple linear regression. The regression equation obtained for fiber tenacity was as follows:
Tenacity, g/d=11.88+2.2211V'+1.147C' +1.948TM' +0.822Q' -1.167L' -2.438DO' +0.532SR -0.7261V'DA' +1.3991V'TM' +0.534lV'L' +0.046lV'SR -0.754C'DA' -0.391C'Q' -0.419C'DO' -1.327D'TM' +0.366D'L' -0.577DA'TM' -0.790DA'Q' -0.034DA'SR -0.049TM'SR +0.809Q'L' -0.313Q'DO'=0.334(IV')2 +0.115(L')² +0.564(DO')² -0.00237(S_{R})²

where:
IV' =(polymer IV, dUg-14.4)/3.1
C' =Gel concentration, %-6
TM'=(spinning temp. °C-200)/20
Q' =(spin flow rate, cc/min-4.38/1.46
L' =(distance to quench, in -15)/9
DO'=1.4427 log (xerogel fiber denier/500)
SR =stretch ratio
(xerogel fiber denier/stretched fiber denier)
DA'=(_{di}e angle, °-7.5)/7.5
D' =(die exit diameter, inches-0.06)/0.02.

The statistics of the regression were:
F ratio (26, 346)=69
Significance Level=99.9+%

Standard error of estimate=2.6 g/denier.

In the vicinity of the center of the experimental space these effects may be summarized by considering the magnitude of change in the factor which is required to increase tenacity of 1 g/d. This is given below.

High fiber tenacity was favored by increasing polymer IV, increasing gel concentration, increasing spinning temperature, decreasing die diameter, decreasing distance to quench, decreasing xerogel fiber diameter, increasing stretch ratio and 0° die angle (straight capillary).

It will be seen that the method of the invention enables substantial control to obtain desired fiber properties and that greater controllability and flexibility is obtained than by prior art methods.

In these experiments, the effects of process parameters upon fiber modulus generally paralled the effects of these variables upon tenacity. Fiber modulus was correlated with tenacity as follows:
modulus, g/d=42(tenacity, g/d) -258

Significance of the correlation between modulus and tenacity was 99.99+%. Standard error of the estimate of modulus was 107 g/d.

It should be noted that many of the fibers of these examples show higher tenacities and/or higher modulus than had seen obtained by prior art methods.

The densities and porosities of several of the xerogel and stretched fibers were determined.

The porosities of these samples were substantially lower than in the prior art methods cited earlier.

### Examples 487-583

In the following Examples of multi-filament spinning and stretching, polymer solutions were prepared as in Example 2. The solutions were spun through a 16 hole spinning die using a gear pump to control solution flow rate. The apertures of the spinning die were straight capillaries of length-to-diameter ratio of 25/1. Each capillary was preceded by a conical entry region of 60° included angle.

The multi-filament solution yarns were quenched to a gel state by passing through a water bath located at a short distance below the spinning die. The gel yarns were wound up on perforated dye tubes.

### Examples 487-495

### One state "dry stretching" of multi-filament yarn

The wound tubes of gel yarn were extracted with TCTFE in a large Sohxlet apparatus to exchange this solvent for paraffin oil as the liquid constituent of the gel. The gel fiber was unwound from the tubes and the TCTFE solvent was evaporated at room temperature.

The dried xerogel yarns were stretched by passing the yarn over a slow speed feed godet and idler roll through a hot tube blanketed with nitrogen, onto a second godet and idler roll driven at a higher speed. The stretched yarn was collected on a winder.

It was noted that some stretching of the yarn (approximately 2/1) occurred as it departed the feed godet and before it entered the hot tube. The overall stretch ratio, i.e., the ratio of the surface speeds of the godets, is given below.

In Examples 487-495, the diameter of each hole of the 16 filament spinning die was 0.040 inch (one millimeter) the spinning temperature was 220°C, the stretch temperature (in the hot tube) was 140°C and the feed roll speed during stretching was 4 cm/min. In Examples 487-490 the polymer IV was 17.5 and the gel concentration was 7 weight %. In Examples 491-495 the polymer IV was 22.6. The gel concentration was 9 weight % in Example 491, 8 weight % in Examples 492-493 and 6 weight % in Examples 494 and 495. The distance from the die face to the quench bath was 3 inches (7.52 cm) in Examples 487, 488, 494 and 495 and 6 inches (15.2 cm) in Examples 490-493. The other spinning conditions and the properties of the final yarns were as follows.

### Examples 496-501

### One stage "wet stretching" of multi-filament yarn

The wound gel yarns still containing the paraffin oil were stretched by passing the yarn over a slow speed feed godet and idler roll through a hot tube blanketed with nitrogen onto a second godet and idler roll driven at high speed. It was noted that some stretching of the yarn (approximately 2/1) occurred as it departed the feed godet and before it entered the hot tube. The overall stretch ratio, i.e., the ratio of the surface speeds of the godets is given below. The stretching caused essentially no evaporation of the paraffin oil (the vapor pressure of the paraffin oil is 0.001 atmospheres at 149°C). However, half of the paraffin oil content of the gel yarns was exuded during stretching. The stretched gel yarns were extracted with TCTFE in a Sohxlet apparatus, then unwound and dried at room temperature.

In each of the Examples 496-501 the spinning temperatures was 220°C, the gel concentration was 6 weight % the distance from the spinning die to the water quench was 3 inches (7.6 cm).

In Examples 496 and 499-501 the diameter of each hole of the spinning die was 0.040 inches (0.1 cm). In Examples 497 and 498 the hole diameters were 0.030 inches (0.075 cm). In Examples 496 and 494-501 the polymer IV was 17.5. In Examples 497 and 498 the polymer IV was 22.6. The other spinning conditions and properties of the final yarns were as follows:

Examples 502-533

In the following Examples a comparison is made between alternative two stage modes of stretching the same initial batch of yarn. All stretching was done in a hot tube blanketed with nitrogen.

### Example 502

### Gel yarn preparation

The gel yarn was prepared from a 6 weight % solution of 22.6 IV polyethylene as in Example 2. The yarn was spun using a 16 holexO.030 inch (0.075 cm) die. Spinning temperature was 220°C. Spin rate was 1 cm³/min-fil. Distance from the die face to the quench bath was 3 inches (7.6 cm). Take-up speed was 308 cm/min. Nine rolls of 16 filament gel yarn was prepared.

### Examples 503-576

### "Wet-wet" stretching

In this mode the gel yarn containing the paraffin oil was stretched twice. In the first stage, three of the rolls of 16 filament gel yarns described in Example 502 above were combined and stretched together to prepare a 48 filament stretched gel yarn. The first stage stretching conditions were: Stretch temperature 120°C, feed speed 35 cm/min, stretch ratio 12/1. A small sample of the first stage stretched gel yarn was at this point extracted with TCTFE, dried and tested for tensile properties. The results are given below as Example 503.

The remainder of the first stage stretched gel yarn was restretched at 1 m/min feed speed. Other second stage stretching conditions and physical properties of the stretched yarns are given below.

The density of the fiber of Example 515 was determined to be 980 kglm^{3.} The density of the fiber was therefore higher than the density of a compression molded plaque and the porosity was essentially zero.

### Examples 517-522

### "Wet-dry" stretching

In this mode the gel yarn was stretched once then extracted with TCTFE, dried and stretched again.

In the first stage, three of the rolls of 16 filament gel yarn described in Example 502 were combined and stretched together to prepare a 48 filament stretched gel yarn. The first stage stretching conditions were: stretch temperature 120°C, feed speed 35 cm/min, stretch ratio 12/1.

The first stage stretched gel yarn was extracted with TCTFE in a Soxhlet apparatus, rewound and air dried at room temperature, then subjected to a second stage of stretching in the dry state at a feed speed of 1 m/min. Other second stage stretching conditions and physical properties of the stretched yarn are given below.

### Examples 523-533

### "Dry-dry" stretching

In this mode the gel yarn described in Example 502 was extracted with TCTFE, dried, then stretched in two stages. In the first stage, three of the rolls of 16 filament yarn were combined and stretched together to prepare a 48 filament stretched xerogel yarn. The first stage stretching conditions were: stretch temperature 120°C, feed speed 35 cm/min., stretch ratio 10/1. The properties of the first stage stretched xerogel yarn are given as Example 523 below. In the second stretch stage the feed speed was 1 m/min. Other second stage stretching conditions and physical properties of the stretched yarns are given below.

The density of the fiber of Example 529 was determined to be 940 Kg/m^{3.} The porosity of the fiber was therefore 2%.

### Examples 534-542

### Multi-stage stretching of multi-filament yarn

In the following Examples a comparison is made between two elevated temperature stretches and a three stage stretch with the first stage at room temperature. The same initial batch of polymer solution was used in these examples.

### Example 534

### Unstretched gel yarn preparation

A 6 weight % solution of 22.6 IV polyethylene yarn was prepared as in Example 2. A 16 filament yarn was spun and wound as in Example 502.

### Example 535

### Preparation of gel yarn stretched at room temperature

The unstretched gel yarn prepared as in Example 534 was led continuously from a first godet which set the spinning take-up speed to a second godet operating at a surface speed of 616 cm/min. In Examples 540-542 only, the as-spun gel fiber was stretched 2/1 at room temperature in-line with spinning. The once stretched gel fiber was wound on tubes.

### Examples 536-542

The 16 filament gel yarns prepared in Examples 534 and 535 were stretched twice at elevated temperature. In the first of such operations the gel yarns were fed at 35 cm/min to a hot tube blanketed with nitrogen and maintained at 120°C. In the second stage of elevated temperature stretching the gel yarns were fed at 1 m/min and were stretched at 150°C. Other stretching conditions and yarn properties are given below.

### Examples 543-551

### Polyethylene yarns of extreme modulus

The highest experimental value reported for the modulus of a polyethylene fiber appears to be by P. J. Barham and A. Keller, J. Poly. Sci., Polymer Letters ed. 17, 591 (1979). The measurement 140 GPa (1587 g/d) was made by a dynamic method at 2.5 Hz and 0.06% strain and is expected to be higher than would be a similar measurement made by A.S.T.M. Method D2101 "Tensile Properties of Single Man Made Fibers Taken from Yarns and Tows" or by A.S.T.M. Method D2256 "Breaking Load (Strength) and Elongation of Yarn by the Single Strand Method". The latter methods were used in obtaining the data reported here.

The following Examples illustrate the preparation of novel polyethylene yarns of modulus exceeding 1600 g/d and in some cases of modulus exceeding 2000 g/d. Such polyethylene fibers and yarns were heretofore unknown. In the following Examples all yarns were made from a 22.6 IV polyethylene, 6 weight % solution prepared as in Example 2 and spun as in Example 502. All yarns were stretched in two stages. The first stage stretch was at a temperature of 120°C. The second stage stretch was at a temperature of 150°C. Several 16 filament yarn ends may have been combined during stretching. Stretching conditions and yarn properties are given below.

The yarns of Examples 548 and 550 were characterized by differential scanning calorimetry at 10°C/min. and density measurement. The results, displayed below, indicate two distinct peaks at the melting points indicated, quite unlike the broad single peak at 145.5°C or less reported by Smith and Lemstra in J. Mat. Sci., vol 15, 505 (1980).

### Examples 552-558

### Polypropylene yarns of extreme modulus

The highest reported experimental value for the modulus of a polypropylene material (fiber or other form) appears to be by T. Williams, J. Mat. Sci., 8, 59 (1973). Their value on a solid state extruded billet was 16.7 GPa (210 g/d). The following Examples illustrate the preparation of polypropylene continuous fibers with modulus exceeding 220 g/d and in some cases of modulus exceeding 250 g/d.

In the following Examples all fibers were made from an 18 IV polypropylene, 6 weight % solution in paraffin oil prepared as in Example 2. In Examples 552-556, the fibers were spun with a single hole conical die of 0.040" (0.1 cm) exit diameter and 7.5% angle. Solution temperature was 220°C. A melt pump was used to control solution flow rate at 2.92 cm³/min. Distance from the die face to the water quench was 3 inches (7.6 cm). The gel fibers were one stage wet stretched at 25 cm/min feed roll speed into a 1.5 m hot tube blanketed with nitrogen. The stretched fibers were extracted in TCTFE and air dried. Other spinning and stretching conditions as well as fiber properties are given below.

The fiber of Example 556 was determined by differential scanning calorimetry at 10°C/min to have a first melting temperature of 170-171°C with higher order melting temperatures of 173°C, 179°C and 185°C. This compares with the 166°C melting point of the initial polymer. The moduli of these fibers substantially exceed the highest previously reported values.

In Examples 557 and 558, the yarns were spun with a 16 holexO.040 inch (1 mm) capillary die. The solution temperature was 223°C, and the spinning rate was 2.5 cm³/min-filament. The distance from the die face to the water quench bath was 3 inches (7.6 cm). Take-up speed was 430 cm/min. The gel yarns were "wet-wet" stretched in two stages. The first stage stretching was at 140°C at a feed speed of 35 cm/min. The second stage stretching was at a temperature of 169°C, a feed speed of 100 cm/min and a stretch ratio of 1.25/1. Other stretching conditions as well as fiber properties are given below.

The moduli of these yarns very substantially exceed the highest previously reported values.

## Claims

1. A continuous process for producing a high strength, high modulus fiber or film which comprises the steps:
(a) forming a solution of a thermoplastic crystalline polymer which is polyethylene of weight average molecular weight at least 500,000 or polypropylene of weight average molecular weight at least 750,000 or which is polyoxymethylene, polybutene-1, poly(vinyledene fluoride) and/or poly(4-methylpentene-I) having a weight average molecular length between 7x10⁴ and 71x10⁴ backbone atoms in a first solvent which is non-volatile at a first temperature, the solution having a first concentration by weight of polymer per unit weight of first solvent;
(b) extruding said solution through an aperture, said solution being at a temperature no less than said first temperature upstream of the aperture and being substantially at the first concentration both upstream and downstream of the aperture;
(c) cooling the emerging stream adjacent to and downstream of the aperture from the first temperature to a second temperature below the temperature at which a rubbery gel stream is formed, including quenching in a quench bath;
(d) extracting the first solvent from the gel stream with a second, volatile solvent;
(e) drying the gel fiber or film containing second solvent to form a continuous xerogel fiber or film free of first and second solvent; and
(f) stretching at least one of:
(i) the gel stream containing the first solvent from step c,
(ii) the gel fiber or film containing the second solvent from step d and,
(iii) the xerogel fiber or film,
at a total stretch ratio:
(i) in the case of polyethylene which is sufficient to achieve a tenacity of at least 20 g/denier (1.7
GPa) and a modulus of at least 600 g/denier (51 GPa),
(ii) in the case of polypropylene which is sufficient to achieve a tenacity of at least 10 g/denier (0.8
GPa) and a modulus of at least 180 g/denier (14 GPa), and
(iii) in the case of polyoxymethylene, polybutene-1, poly(vinylidene fluoride) or poly(4-methylpentene-1) of at least 10:1.

2. The process of claim 1 wherein said aperture has an essentially circular cross-section and the product is a fiber.

3. The process of claim 1 or 2 wherein said first temperature is between 150°C and 250°C; said second temperature is between -40°C and 40°C; the cooling rate between said first temperature and said second temperature is at least 50°C/min; and said first solvent is a hydrocarbon.

4. The process of any previous claim wherein said first solvent has a vapor pressure less than 20 kPa at said first temperature and said second solvent is non-flammable and has an atmospheric boiling point less than 80°C.

5. The process of any previous claim wherein said second solvent has an atmospheric boiling point less than 50°C.

6. The process of any previous claim wherein said stretching step (f) is conducted in at least two stages.

7. The process of any previous claim wherein the thermoplastic crystalline polymer is polyethylene and at least a portion of stretching is performed at a temperature between 120°C and 160°C.

8. The process of claim 7 wherein the stretching is performed in at least two stages with the latest stage performed at a temperature of between 135°C and 150°C.

9. A continuous polyethylene fiber of weight average molecular weight at least 500,000 and having a tenacity of at least 20 g/denier (1.7 GPa) and a tensile modulus at least 500 g/denier (43 GPa), characterized by having a creep value no more than 5% (when measured at 10% of breaking load for 50 days at 23°C), a porosity less than 10% and a main melting temperature of at least 147°C (measured by DSC at 10 °C/minute heating rate).

10. The polyethylene fiber of claim 9 having a tenacity of at least 30 g/denier (2.56 GPa) and a tensile modulus of at least 1000 g/denier (85.6 GPa).

11. The polyethylene fiber of claim 9 or 10 having a tensile modulus of at least 1600 g/denier (137 GPa).

12. The polyethylene fiber of claim 11 having a tensile modulus of at least 2000 g/denier (171 GPa).

13. The polyethylene fiber of claim 9 or 10 or 11 or 12 being of weight average molecular weight between 2,000,000 and 8,000,000.

14. The polyethylene fiber of any of claims 9-13 having an elongation-to-break of not more than 5%.

15. A continuous polypropylene fiber of weight average molecular weight at Ieast 750,000 and having a tenacity of at least 8 g/denier (0.6 GPa), characterized by having a tensile modulus of at least 160 g/denier (13.7 GPa) and a main melting temperature of at least 168°C (measured by DSC at 10°C/minute heating rate).

16. The polypropylene fiber of claim 15 having a tensile modulus of at least 220 g/denier (17.6 GPa).

17. The polypropylene fiber of claim 15 or 16 being of weight average molecular weight between 2,000,000 and 8,000,000.

18. A continuous polyolefin gel fiber comprising between 4 and 20 weight % solid polyethylene of weight average molecular weight at least 500,000 or solid polypropylene of weight average molecular weight at least 750,000, and between 80 and 96 weight % of a swelling solvent miscible with a high boiling hydrocarbon, characterized by the swelling solvent having an atmospheric boiling point less than 50°C.

## Patentansprüche

1. Kontinuierliches Verfahren zum Erzeugen einer Faser oder eines Films von hoher Festigkeit und hohem Elastizitätsmodul, mit folgenden Schritten:
(a) Es wird eine Lösung eines thermoplastischen kristallinen Polymers gebildet, das aus Polyethylen mit einem gewichtsdurchschnittlichen Molekulargewicht von mindestens 500 000 oder aus Polypropylen mit einem gewichtsdurchschnittlichen Molekulargewicht von mindestens 750 000 oder aus Polyoxymethylen, Polybuten-1, Poly(vinylidenfluorid) und/oder Poly(4-methylpenten-1) mit einer gewichtsdurchschnittlichen Moleküllänge zwischen 7× 10° und 71 x 10⁴ Atomen in der Hauptkette in einem ersten Lösungsmittel hergestellt, das bei einer ersten Temperatur nichtflüchtig ist, wobei die Lösung eine erste Gewichtskonzentration des Polymers pro Gewichtseinheit des ersten Lösungsmittels besitzt;
(b) die Lösung wird durch ein Öffnung extrudiert, wobei sich die Lösung stromauf der Öffnung auf einer Temperatur befindet, die nicht niedriger ist als die erste Temperatur, und die Lösung sowohl stromauf als auch stromab der Öffnung im wesentlichen die erste Konzentration hat,
(c) der austretende Strom wird im Bereich der Öffnung und stromab von ihr von der ersten Temperatur auf eine zweite Temperatur abgekühlt, die niedriger ist als die Temperatur, bei der sich ein kautschukartiger Gelstrom bildet, wobei in einem Abschreckbad abgeschreckt wird;
(d) das erste Lösungemittel wird aus dem Gel mit einem flüchtigen zweiten Lösungsmittel extrahiert,
(e) durch Trocknen des das zweite Lösungsmittel enthaltenden, faser- oder filmförmigen Gels wird ein kontinuierliches faser- oder filmförmiges Xerogel gebildet, das von dem ersten und dem zweiten Lösungsmittel frei ist, und
(f) mindestens eine der Substanzen:
(i) der im Schritt c erhaltene, das erste Lösungsmittel enthaltende Gelstrom;
(ii) das im Schritt d erhaltene, das zweite Lösungsmittel enthaltende, faser- oder filmförmige Gel und
(iii) das faser- oder filmförmige Xerogel;
wird mit einem Gesamtstreckverhältnis gestreckt, das
(i) bei Polyethylen genügt, um eine Reißfestigkeit von mindestens 0 g/den (1,7 GPa) und einen Elastizitätsmodul von mindestens 600 g/den (51 GPa) zu erzielen,
(ii) bei Polypropylen genügt, um eine Reißfestigkeit von mindestens 10 g/den (0,8 GPa) und einen Elastizitätsmodul von mindestens 180 g/den (14 GPa) zu erzielen, und
(iii) bei Polyoxymethylen, Polybuten-1, Poly(vinylidenfluorid) oder Poly(4-methylpenten-1) mindestens 10:1 beträgt.

2. Verfahren nach Anspruch 1, dadurch gekennzeichnet, daß die Öffnung im Querschnitt im wesentlichen kreisförmig und das Produkt eine Faser ist.

3. Verfahren nach Anspruch 1 oder 2, dadurch gekennzeichnet, daß die erste Temperatur zwischen 150 und 250°C, die zweite Temperatur zwischen -40 und 40°C und die Abkühlungsgeschwindigkeit zwischen der ersten und der zweiten Temperatur mindestens 50°C/min begrägt und daß das erste Lösungsmittel ein Kohlenwasserstoff ist.

4. Verfahren nach einem der vorhergehenden Ansprüche, dadurch gekennzeichnet, daß das erste Lösungsmittel bei der ersten Temperatur einen Dampfdruck von weniger als 20 kPa hat und daß das zweite Lösungsmittel nichtentflammbar ist und unter atmosphärischem Druck einen Siedepunkt unter 80°C hat.

5. Verfahren nach einem der vorhergehenden Ansprüche, dadurch gekennzeichnet, daß das zweite Lösungsmittel unter atmosphärischem Druck einen Siedepunkt unter 50°C hat.

6. Verfahren nach einem der vorhergehenden Ansprüche, dadurch gekennzeichnet, daß der Streckschritt (f) in mindestens zwei Stufen durchgeführt wird.

7. Verfahren nach einem der vorhergehenden Ansprüche, dadurch gekennzeichnet, daß das thermoplastische kristalline Polymer Polyethylen ist und das Strecken mindestens zum Teil bei einer Temperatur zwischen 120 und 160°C durchgeführt wird.

8. Verfahren nach Anspruch 7, dadurch gekennzeichnet, daß das Strecken in mindestens zwei Stufen und die letzte Stufe bei einer Temperatur zwischen 135 und 150°C durchgeführt wird.

9. Polyethylen-Endlosfaser mit einem gewichtsdurchschnittlichen Molekulargewicht von mindestens 500 000, einer Reißfestigkeit von mindestens 20 g/den (1,7 GPa) und einem Elastizitätsmodul von mindestens 500 g/den (43 GPa), dadurch gekennzeichnet, daß sie einen (bei Belastung mit 10% der Brucklast für 50 Tage bei 23°C gemessenen) Kriechwert von nicht mehr als 5%, eine Porosität von 10% und eine durch Kalorimetrie mit differentieller Abtastung (bei einer Erhitzungsgeschwindigkeit von 10°C/min gemessene) Hauptschmelztemperatur von mindestens 147°C hat.

10. Polyethylenfaser nach Anspruch 9 mit einer Reißfestigkeit von mindestens 30 g/den (2,56 GPa) und einem Elastizitätsmodul von mindestens 1000 g/den (85,6 GPa).

11. Polyethylenfaser nach Anspruch 9 oder 10 mit einem Elastizitätsmodul von mindestens 1600 g/den (137 GPa).

12. Polyethylenfaser nach Anspruch 11 mit einem Elastizitätsmodul von mindesten- 2000 g/den (171 GPa).

13. Polyethylenfaser nach Anspruch 9, 10, 11 oder 12, mit einem gewichtsdurchschnittlichen Molekulargewicht zwischen 2000000 und 8000000.

14. Polyethylenfaser nach einem der Ansprüche 9 bis 13, mit einer Bruchdehnung von nicht mehr als 5%.

15. Polypropylen-Endlosfaser mit einem gewichtsdurchschnittlichen Molekulargewicht von mindestens 750 000 und einer Reißfestigkeit von mindestens 8 g/den (0,6 GPa), dadurch gekennzeichnet, daß sie einen Elastizitätsmodul von mindestens 160 g/den (13,7 GPa) und eine (durch Kalorimetrie mit differentieller Abtastung bei einer Erhitzungsgeschwindigkeit von 10°C/min gemessene) Hauptschmelztemperatur von mindestens 168°C hat.

16. Polypropylenfaser nach Anspruch 15 mit einem Elastizitätsmodul von mindestens 220 g/den (17,6 GPa).

17. Polypropylenfaser nach Anspruch 15 oder 16 mit einem gewichtsdurchschnittlichen Molekulargewicht zwischen 2 000 000 und 8 000 000.

18. Polyolefingel-Endlosfaser mit einem Gehalt von 4 bis 20 Gew.% festem Polyethylen, das ein gewichtsdurchschnittliches Molekulargewicht von mindestens 500 000 hat, oder festem Polypropylen, das ein gewichtsdurchschnittliches Molekulargewicht von mindestens 750 000 hat, und mit einem Gehalt von 80 bis 96 Gew.% eines quellend wirkenden Lösungsmittels, das mit einem hochsiedenden Kohlenwasserstoff mischbar ist, dadurch gekennzeichnet, daß das quellend wirkende Lösungsmittel unter atmosphärischem Druck einen Siedepunkt unter 50°C hat.

## Revendications

1. Procédé continu pour produire une fibre ou un film à haute résistance et module élevé, qui comprend les stades:
a) de former une solution d'un polymère cristallin thermoplastique qui est du polyéthylène d'un poids moléculaire moyen en masse d'au moins 500.000 ou du polypropylène d'un poids moléculaire moyen en masse d'au moins 750.000 ou qui est du polyoxyméthylène, du polybutène-1, du poly(fluorure de vinylidène) et/ou du poly(4-méthylpentène-1) ayant une longueur moléculaire moyenne en masse entre 7x104 et 71 x104 atomes de squelette dans un premier solvant qui est non volatil à une première température, la solution ayant une première concentration en poids de polymère par unité de poids du premier solvant;
b) d'extruder la solution à travers un orifice, la solution étant à une température non inférieure à cette première température à l'amont de l'orifice et étant sensiblement à la première concentration tant à l'amont qu'à l'aval de l'orifice;
c) de refroidir le courant émergeant au voisinage et à l'aval de l'orifice à partir de la première température jusqu'à une seconde température inférieure à la température à laquelle un courant de gel caoutchouteux est formé, notamment de tremper dans un bain de trempe;
d) d'extraire le premier solvant du courant de gel au moyen d'un second solvant qui est volatile;
e) de sécher la fibre ou le fil de gel contenant le second solvant pour former une fibre ou un film de xérogel continu exempt du premier solvant et du second; et
f) d'étirer au moins l'un d'entre:
(i) le courant de gel contenant le premier solvant du stade c,
(ii) la fibre ou le film de gel contenant le second solvant du stade d et,
(iii) la fibre ou le film de xérogel,
à un rapport d'étirage total:
(i) dans le cas du polyéthylène, qui est suffisant pour atteindre une ténacité d'au moins 20 g/denier (1,7 GPa) et un module d'au moins 600 g/denier (51 GPa).
(ii) dans le cas du polypropylène, qui est suffisant pour atteindre unt ténacité d'au moins 10 g/denier (0,8 GPa) et un module d'au moins 180 g/denier (1 GPa), et
(iii) dans le cas du polyoxyméthylène, du polybutène-1, du poly(fluorure de vinylidène) ou du poly(4-méthylpentène-1), d'au moins 10:1.

2. Procédé suivant la revendication 1, dans lequel l'orifice présente une section sensiblement circulaire et le produit est une fibre.

3. Procédé suivant la revendication 1 ou 2, dans lequel la première température est entre 150°C et 250°C et la seconde température est entre -40°C et 40°C, l'allure de refroidissement entre la première température et la seconde température est d'au moins 50°C/minute et le premier solvant est un hydrocarbure.

4. Procédé suivant l'une quelconque des revendications précédentes, dans lequel le premier solvant a une tension de vapeur inférieure à 20 kPa à la première température et le second solvant est ininflammable et a un point d'ébullition atmosphérique inférieur à 80°C.

5. Procédé suivant l'une quelconque des revendications précédentes, dans lequel le second solvant a un point d'ébullition atmosphérique inférieur à 50°C.

6. Procédé suivant l'une quelconque des revendications précédentes, dans lequel le stade d'étirage (f) est exécuté en au moins deux étapes.

7. Procédé suivant l'une quelconque des revendications précédentes, dans lequel le polymère cristallin thermoplastique est le polyéthylène et au moins une partie de l'étirage est exécutée à une température entre 120°C et 160°C.

8. Procédé suivant la revendication 7, dans lequel l'étirage est exécuté en au moins deux étapes, la dernière étape étant exécutée à une température entre 135°C et 150°C.

9. Fibre de polyéthylène continue d'un poids moléculaire moyen en masse d'au moins 500.000 et ayant une ténacité d'au moins 20 g/denier (1,7 GPa) et un module de traction d'au moins 500 g/denier (43 GPa), caractérisée en ce qu'elle a une valeur de fluage n'excédant pas 5% (mesurée à 10% de la charge de rupture pendant 50 jours à 23°C), une porosité inférieure à 10% et une température de fusion principale d'au moins 147°C (mesurée par ATD à une allure de chauffage de 10°C/minute).

10. Fibre de polyéthylène suivant la revendication 9, ayant une ténacité d'au moins 30 g/denier (2,56 GPa) et un module de traction d'au moins 1000 g/ denier (85,6 GPa).

11. Fibre de polyéthylène suivant la revendication 9 ou 10, ayant un module de traction d'au moins 1600 g/denier (137 GPa).

12. Fibre de polyéthylène suivant la revendication 11, ayant un module de traction d'au moins 2000 g/denier (171 GPa).

13. Fibre de polyéthylène suivant la revendication 9 ou 10 ou 11 ou 12, ayant un poids moléculaire moyen en masse entre 2.000.000 et 8.000.000.

14. Fibre de polyéthylène suivant l'une quelconque des revendications 9-13, ayant un allongement à la rupture n'excédant pas 5%.

15. Fibre de polypropylène continue d'un poids moléculaire moyen en masse d'au moins 750.000 et ayant une ténacité d'au moins 8 g/denier (0,6 GPa), caractérisée en ce qu'elle a un module de traction d'au moins 160 g/denier (13,7 GPa) et une température de fusion principale d'au moins 168°C (mesurée par ATD à une allure de chauffage de 10°C/minute).

16. Fibre de polypropylène suivant la revendication 15, ayant un module de traction d'au moins 220 g/denier (17,6 GPa).

17. Fibre de polypropylène suivant la revendication 15 ou 16, ayant un poids moléculaire moyen en masse entre 2.000.000 et 8.000.000.

18. Fibre de gel de polyoléfine continue comprenant entre 4 et 20% en poids de polyéthylène solide d'un poids moléculaire moyen en masse d'au moins 500.000 ou de polypropylène solide d'un poids moléculaire moyen en masse d'au moins 750.000 et entre 80 et 96% en poids d'un solvant de gonflement miscible avec un hydrocarbure à haut point d'ébullition, caractérisée en ce que le solvant de gonflement a un point d'ébullition atmosphérique inférieur à 50°C.
